

1

3,331,797  
FLAME-RESISTANT POLYOLEFINE  
COMPOSITIONS

Kurt Kopetz and Fritz Baxmann, Marl, Germany, assignors to Chemische Werke Huls Aktiengesellschaft, Marl, Germany, a corporation of Germany  
No Drawing. Filed Feb. 12, 1964, Ser. No. 344,244  
2 Claims. (Cl. 260—28.5)

Due to their ready flammability polyolefines such as polyethylene, polypropylene and polyisobutylene cannot be used as such in the construction and other fields in which difficultly flammable materials are required. It has been attempted, therefore to render polyolefines flame resistant by additions of chloroparaffines in conjunction with antimony trioxide. Satisfactorily flame resistant products are however not obtainable by such additions if the amount of the addition is sufficiently small that other essential properties, especially strength are not unfavorably affected. The great disadvantage of chloroparaffine additions lies in the fact that these compounds, even at relatively low temperatures, tend to liberate hydrogen chloride which attacks the machines used in working and forming the composition. The amount of addition required to give a relatively satisfactory flame resistant polyolefine is, in any case, more than 20%. It is not feasible to add sufficient acid acceptor to compositions containing such a high content of chloroparaffine to effect an adequate stabilization.

The use of nucleus bromine substituted aromatic compounds as disclosed in e.g., German Patents Nos. 1,103,020, 1,123,823, 1,127,582 and 1,135,653 brought about a decisive improvement particularly in the avoidance of the difficulties associated with the use of chloroparaffines.

The testing of the material in the form of plates with respect to flame resistance, self-extinguishment and burning is carried out in two ways as follows:

(1) DIN 4102, page 1

4 plates having the dimensions 1000 x 190 x 3 mm. are supported vertically and in a chimney-like arrangement at right angles to each other and hung in a shaft furnace. Air is passed upwardly through a sieve bottom. Flame is generated by a ring burner having 36 nozzle openings so that the flame strikes the inner surfaces of the plates. The length of the flame is about 250–300 mm. After 11 minutes of the flame treatment the burning of the plates must extinguish immediately or in a short time and at least 15% of the plates must remain undamaged.

(2) ASTM D635-56T

A test piece having the dimensions 127 x 12.7 x 3 mm. is supported at an angle of 45° to its horizontal axis. It is then flamed with a Bunsen burner having a diameter of 5 mm. and with a flame about 12 to 13 mm. long with the tip of the flame just reaching the lower end of the test body. The flaming time is 2 to 30 seconds. If the sample does not continue to burn after removal of the flame it is classified as "non-burning by this test." If the

2

sample continues to burn after the removal of the flame but not beyond the 4 inch-marking it is classified as "self-extinguishing by this test." If the test piece continues to burn after removal of the flame it is classified as "burning by this test."

In the DIN test the burning conditions are such as to correspond to a fire storm, that is, very high temperatures which are increased by the heat of combustion of the sample itself and by the chimney arrangement of the test pieces. Under such conditions only such additions are effective as are effective at relatively high temperatures. Such compounds are for example the above mentioned aromatic bromine compounds. Aliphatic chlorine compounds are completely useless under these conditions because the decomposition temperature of this type of compounds is very low. The addition of stabilizers does not change this situation. In general it can be assumed that the flaming of differently burnable polyolefines first forms hydrogen chloride which can stop or interrupt the chain reaction of the burning. This action in most cases is increased by antimony trioxide.

The course of the combustion is quite different in the ASTM test process. Here a relatively small flame is used and the mass and energy content of the test body is small. Under these conditions it can be expected that added flame-proofing material having a relatively high decomposition range cannot be effective since the burning temperature of the synthetic resin body does not at all or only to an insufficient extent affect the addition material.

There is a strong technical interest in the provision of an addition or addition mixture which is effective under all practically occurring burning conditions and is equally effective in both test methods.

It has now been found that flame resistant polyolefine mixtures which contain from 5 to 20% by weight of nucleus brominated aromatic compounds, 2 to 10% by weight of chlorinated paraffines and 2 to 9% by weight of antimony trioxide are especially useful.

Suitable polyolefines for use in the compositions are polyethylene, polypropylene, polyisobutylene and the solid mixed polymers of the corresponding monomers. The polyolefines may contain the usual additions of fillers, colors, lubricants, and/or stabilizers.

Suitable nucleus brominated aromatic compounds that are to be incorporated into the mixtures in amounts from 5 to 20% preferably from 5 to 12% and especially from 5 to 9% by weight, based upon the polyolefine content of the mixture, are the aromatic compounds containing at least three bromine atoms in the nucleus, of the general formulae



and



in which  $R_1$  to  $R_{10}$  stand for hydrogen, bromine, chlorine, methyl, straight chain and branched chain alkyl and alkenyl groups having from 2 to 4 carbon atoms and the benzyl group which may be substituted by bromine, chlorine or both,  $X$  stands for a divalent saturated or unsaturated aliphatic group which may be substituted by bromine and/or chlorine or one or more aromatic groups, so many of  $R_1$  to  $R_{10}$  standing for bromine that they together with any other bromine atoms attached to an aromatic nucleus in the molecule amount to at least 3 bromine atoms that are bound directly to an aromatic nucleus. Examples of the values of  $X$  are the methylene, ethylidene, propylidene, dimethylmethylen, ethylene, trimethylene, vinylidene, vinylene and allylidene groups. The compounds should contain a total of from 50 to 85% by weight of bromine; from 0 to 30% by weight of this bromine may be substituted by chlorine. The distribution of the halogen atoms on the aromatic ring is optional.

Examples of nucleus halogenated diaromatic compounds are the halogenation products of dibenzyl, dimethylbenzyl, diethylbenzyl, benzyltoluene, dibenzyltoluene, benzylmethyl-benzylbenzene, diphenylpropane, diphenyls and their mixtures. These compounds need not exhibit any particular stoichiometry. On the contrary it may be advantageous to use mixtures of compounds just as they are produced by halogenation of the named starting materials or mixtures thereof without fractionation or separation in any manner. These mixtures of compounds which are mostly of oily or colophony-like consistency contain different numbers and different arrangements of the halogen atoms and generally have less tendency to crystallize than pure compounds. This facilitates the working up of the polyolefine mixtures.

Diaromatic or aromatic-aliphatic ethers containing at least three nucleus substituted bromine atoms of the following formula



may be used. In this formula  $R_1$  stands for an aromatic group that may be brominated and/or chlorinated or a straight or branched chain alkyl group having from 2 to 12 carbon atoms and which may contain a hydroxyl group and  $R_2$  to  $R_6$  stand for hydrogen, chlorine or bromine, there being at least three aromatic nucleus-bound bromine atoms per molecule counting those represented by  $R_2$  to  $R_6$  and those present, if any, on the group represented by  $R_1$ .

Examples of diaromatic ethers having bromine bound to an aromatic nucleus are tribromodiphenyl ether, tetrabromodiphenyl ether, pentabromodiphenyl ether, hexabromodiphenyl ether, tribromomonochloride-diphenyl ether, tribromodichloride-diphenyl ether, tribromotrichloride-diphenyl ether, and tetrabromodichloride-diphenyl ether. The halogen atoms of these diaromatic ethers can be distributed at random on the aromatic rings. Examples of suitable aromatic-aliphatic ethers are the 2-ethylhexyl-, n-octyl, nonyl-, butyl-, dodecyl-, and 2,3-dioxypropyl ethers of tribromophenol, tribromomonochlorophenol and tribromodichlorophenol.

Also nucleus brominated, multinuclear aromatic amines may be used which contain from 50 to 85% by weight of halogen of which 50 to 85% by weight is bromine and from 0 to 30% by weight is chlorine and which contain at least 3 bromine atoms per molecule bound to an aromatic ring. These compounds may contain a total

of from 1 to 4 straight chain or branched chain alkyl groups having from 1 to 4 carbon atoms which may contain OH— groups, substituted on the aromatic rings and possibly also on the nitrogen atoms. Examples of suitable nucleus brominated multinuclear aromatic amines are the corresponding halogenation products of diphenylamine,  $\alpha$ -naphthylamine,  $\beta$ -naphthylamine, 1,1-dinaphthylamine and 1,2-dinaphthylamine. In the bromination it may be advantageous to substitute a part of the bromine by chlorine provided that at least three bromine atoms are bound to an aromatic ring and the total bromine content of the molecule is at least 50% by weight. The halogen in excess of three bromine atoms per molecule may occupy any desired position. It is especially advantageous to use the crude halogenation products which generally are mixtures of isomeric compounds of different halogen contents. The crude halogenation mixtures are generally compatible with the polyolefines as chemically homogeneous compounds.

Another group of suitable compounds are the 2,4,6-tribromoanilines of the formula



in which  $R_1$  and  $R_2$  stand for hydrogen, acyl groups or alkyl groups having from 1 to 6 carbon atoms and  $R_3$  and  $R_4$  stand for hydrogen or alkyl groups having from 1 to 6 carbon atoms. This group of compounds includes 2,4,6-tribromoaniline itself as well as 2,4,6-tribromoanilines substituted in the nucleus and/or on the nitrogen such as 2,4,6-tribromoacetanilide and 2,4,6-tribromolauroylanilide.

Suitable chloroparaffines are the chlorinated straight chain or branched chain or cyclical paraffines having a chlorine content of from 40 to 80%, by weight, preferably 50 to 70%. The chlorinated paraffines are used in amounts within the range from 2 to 10%, preferably 2-5%, by weight, based upon the polyolefine.

Antimony trioxide is used in amounts within the range from 3 to 10%, preferably 4-8%, by weight, based upon the polyolefine.

The components can be mixed with the polyolefine singly in any order or all together and incorporated in known manner. The resulting mixtures are formed or molded in known manner.

It is surprising that the small additions of chlorinated paraffines which alone are not effective by any test method so activate the aromatic, nucleus-substituted compounds that they are effective even at low burning temperatures.

The small amounts of chlorinated paraffines used may be stabilized with the commercially available stabilizers as is customary in the working up of polyvinyl chloride, sufficient stabilizer being used so that at the temperature necessary for working up the polyolefines no corrosion of the machine and molds will result from the splitting off of hydrogen chloride.

The claimed mixture exhibits not only the expected but also a highly valuable synergistic effect.

In the following examples plates having the dimensions 300 x 70 x 3 mm, were subjected to the burning test in accordance with the specifications DIN 4102. The plates were heated in a shaft furnace with practically colorless Bunsen flame, 15 mm. long for 4 minutes. In the examples the amounts of the ingredients of the compositions are given in parts by weight.

| Ex. |                                                                                                                                                                                                                              | Test on the plates | Test According to ASTM D635 | Observation                                        |
|-----|------------------------------------------------------------------------------------------------------------------------------------------------------------------------------------------------------------------------------|--------------------|-----------------------------|----------------------------------------------------|
| 1   | 100 polyethylene (mol. wt. about 40,000), 10 pentabromomonochlorodiphenyl ether, 5 antimony trioxide.                                                                                                                        | Standing           | Self-extinguishing          | Dripping material continues burning for some time. |
| 2   | 100 polyethylene (mol. wt. about 40,000), 7 pentabromomonochlorodiphenyl ether, 5 antimony trioxide.                                                                                                                         | Not standing       | Burning                     | Dripping material continues burning.               |
| 3   | 100 polyethylene (mol. wt. about 40,000), 3 chloroparaffine (chlorine content 70%), 5 antimony trioxide.                                                                                                                     | do                 | do                          | Do.                                                |
| 4   | 100 polyethylene (mol. wt. about 40,000), 7 pentabromomonochlorodiphenyl ether, 3 chloroparaffine (chlorine content 70%), 5 antimony trioxide.                                                                               | Standing           | Not burning                 | Dripping material extinguishes immediately.        |
| 5   | 100 polypropylene (mol. wt. about 300,000), 10 tribromoacetanilide, 5 antimony trioxide.                                                                                                                                     | Almost standing    | Burning                     | Dripping material burns a short time.              |
| 6   | 100 polypropylene (mol. wt. about 300,000), 4 chloroparaffine (chlorine content 70%), 5 antimony trioxide.                                                                                                                   | Not standing       | do                          | Dripping material continues burning.               |
| 7   | 100 polypropylene (mol. wt. about 300,000), 4 chloroparaffine (chlorine content 70%), 9 tribromoacetanilide, 5 antimony trioxide.                                                                                            | Standing           | Not burning                 | Dripping material extinguishes immediately.        |
| 8   | 100 ethylene-propylene mixed polymer (mol. wt. about 50,000), 8 nucleus brominated dibenzyl-toluene-benzyl-methylbenzylbenzene mixture (bromine content 64%), 4 antimony trioxide.                                           | Not standing       | Burning                     | Dripping material burns a short time.              |
| 9   | 100 ethylene-propylene mixed polymer (mol. wt. about 50,000), 4 chloroparaffine (chlorine content 65%), 4 antimony trioxide.                                                                                                 | do                 | do                          | Dripping material continues to burn.               |
| 10  | 100 ethylene-propylene mixed polymer (mol. wt. about 50,000), 7 nucleus brominated dibenzyl-toluene-benzyl-methylbenzylbenzene mixture (bromine content 64%), 4 chloroparaffine (chlorine content 70%), 4 antimony trioxide. | Standing           | Not burning                 | Dripping material extinguishes immediately.        |
| 11  | 100 polyethylene (mol. wt. about 90,000), 10 halogenated diphenylamine (bromine content 62%), chlorine content 3%, 5 antimony trioxide.                                                                                      | do                 | Burning                     | Dripping material burns for a time.                |
| 12  | 100 polyethylene (mol. wt. about 90,000), 10 halogenated diphenylamine (bromine content 62%, chlorine content 3%), 4 chloroparaffine (chlorine content 70%), 4 antimony trioxide.                                            | do                 | Not burning                 | Dripping material extinguishes immediately.        |
| 13  | 100 polyethylene (mol. wt. about 90,000), 4 chloroparaffine (chlorine content 70%), 4 antimony trioxide.                                                                                                                     | Not standing       | Burning                     | Dripping material continues to burn.               |
| 14  | 100 polybutene-1, 10 pentabromomonochlorodiphenyl ether, 5 antimony trioxide.                                                                                                                                                | do                 | Self extinguishing          | Dripping material burns for a time.                |
| 15  | 100 polybutene-1, 7 pentabromomonochlorodiphenyl ether, 5 antimony trioxide.                                                                                                                                                 | Not standing       | Burning                     | Dripping material continues to burn.               |
| 16  | 100 polybutene-1, 3 chloroparaffine (chlorine content 70%), 5 antimony trioxide.                                                                                                                                             | do                 | do                          | Do.                                                |
| 17  | 100 polybutene-1, 7 pentabromomonochlorodiphenyl ether, 3 chloroparaffine (chlorine content 70%), 5 antimony trioxide.                                                                                                       | Standing           | Not standing                | Dripping material extinguishes immediately.        |

In Examples 4, 7, 10 and 17 similar results are obtainable by using bromine- or chlorine-bromine-substituted dibenzyl, dimethyldibenzyl, diethyldibenzyl, benzyltoluene, diphenyl, diphenylmethane, diphenylethane, diphenylpropane, diphenyl ether, diphenylamine or naphthylamine having from 3 to 8 bromine atoms and from 1 to 3 chlorine atoms per molecule as the aromatic bromine-chlorine containing compound.

We claim:

1. A flame resistant polyolefine composition consisting essentially of a normally solid polyolefine, from 2 to 10% by weight, based on the weight of the polyolefine of a chlorinated paraffine, from 2 to 12% by weight based on the weight of the polyolefine of antimony trioxide and from 5 to 20% by weight based on the weight of the polyolefine of a nucleus brominated aromatic compound containing at least three bromine atoms per molecule bound directly to an aromatic nucleus and containing from 50 to 85% by weight of halogen of which from 50 to 85% by weight is bromine and from 0 to 30% by weight is chlorine, at least 50% by weight of the molecule being bromine, said compound being selected from the group consisting of (1) compounds of the formulae



and



in which  $R_1$  to  $R_{10}$  each stands for a member selected from the group consisting of hydrogen, bromine, chlorine, methyl, straight chain and branched chain alkyl and alkenyl groups having from 2 to 4 carbon atoms and the benzoyl group which may be substituted by at least one halogen selected from the group consisting of bromine and chlorine,  $X$  stands for a member selected from the group consisting of divalent saturated and unsaturated aliphatic groups which may be substituted by at least one member selected from the group consisting of bromine, chlorine and aromatic groups; (2) compounds of the formula



in which  $R_1$  stands for a member selected from the group consisting of aromatic groups that may contain at least one halogen selected from the group consisting of bromine and chlorine, straight and branched chain alkyl groups having from 2 to 12 carbon atoms and which may contain hydroxyl groups and  $R_2$  to  $R_8$  each stands for a member selected from the group consisting of hydrogen, chlorine and bromine; (3) multinuclear aromatic amines containing from 1 to 4 alkyl groups each having from 1 to 4 carbon atoms which may contain OH groups; and (4) compounds of the formula



in which  $R_1$  and  $R_2$  each stands for a member selected from the group consisting of hydrogen, acyl groups and alkyl groups having from 1 to 6 carbon atoms and  $R_3$  and  $R_4$  each stands for a member selected from the group consisting of hydrogen and alkyl groups having from 1 to 6 carbon atoms.

2. A flame resistant polyolefine composition as defined in claim 1 in which the nucleus brominated aromatic compound contains from 50 to 85% by weight of bromine and the chlorinated paraffine contains from 40 to 10 80% by weight of chlorine.

## References Cited

## UNITED STATES PATENTS

|           |         |              |          |
|-----------|---------|--------------|----------|
| 2,962,464 | 11/1960 | Feild        | 260—28.5 |
| 3,075,944 | 1/1963  | Wick         |          |
| 3,093,599 | 6/1963  | Mueller-Tamm |          |
| 3,250,739 | 5/1966  | Sauer        |          |

MORRIS LIEBMAN, Primary Examiner.

JULIUS FROME, Examiner.